

Mar. 6, 1923.

1,447,750

C. S. BIRD

SHINGLE

Filed Mar. 3, 1920

*Fig. 1.*



*Fig. 2.*



Inventor

Charles S. Bird  
By Dodge and Dow,  
Attorneys

Patented Mar. 6, 1923.

1,447,750

# UNITED STATES PATENT OFFICE.

CHARLES S. BIRD, OF EAST WALPOLE, MASSACHUSETTS.

## SHINGLE.

Application filed March 3, 1920. Serial No. 363,039.

To all whom it may concern:

Be it known that I, CHARLES S. BIRD, a citizen of the United States, residing at East Walpole, in the county of Norfolk and State 5 of Massachusetts, have invented certain new and useful Improvements in Shingles, of which the following is a specification.

This invention pertains to so-called felt or paper shingles, and has for one of its objects the provision of means for preventing the shingles from adhering or sticking to one another when stacked or placed in bundles. The invention has for its further object the rendering of the under face of the 15 shingle adjacent its lower edge waterproof.

Felt shingles as now commonly made are produced from felt stock cut to size and form and impregnated and coated with asphaltum or similar material in order to 20 render them weather-resistant. Asphaltum is more or less sticky or tacky and when the shingles are stacked or placed in bundles the asphaltum coating which is sometimes applied to the under face of the shingle causes 25 the shingles to stick together unless, perchance, the bundles are packed in wooden crates which relieves them of facewise pressure to a considerable extent. Wooden crating, however, is too expensive to consider 30 from a commercial point of view, and as a consequence the present invention has to deal with the treatment of the under face of the shingle with a waterproofing material which not only waterproofs the shingle but 35 prevents the superimposed shingles from adhering together when bound in bundles.

The invention is sought to be illustrated in the annexed drawings, wherein,—

Fig. 1 is a perspective view of one of the 40 shingles, as seen from the under side; and

Fig. 2 shows a plurality of shingles im- 45 posed one upon the other.

In the drawing, 1 denotes the shingle body which may be of any form and composed of 45 one or more layers of felt stock or the like pressed together and impregnated with asphaltum or any other suitable weather-resistant material. The shingle from the lower edge and upon its under face will 50 have applied thereto a coating, as 2, of a non-sticky substance, and preferably of a waxy nature, such, for instance as Montan wax. This coating is applied for a distance of 4½ inches, more or less, from the lower 55 edge or butt toward the upper edge of the shingle and will prevent that portion of the

shingle from sticking to the next adjacent underlying shingle of the bundle. Such distance or extent is equal, or approximately so, to the exposed area of the shingles 60 when laid.

Felt shingles as now commonly employed, are usually provided upon that face which is exposed when the shingles are laid, with a finish surface 3, formed from comminuted 65 stone or rock, which is colored or has an inherent color, such material being forced into the face of the shingle and caused to adhere thereto by a suitable substance having a cementitious action. Such surface, or at 70 least the portion thereof which is left exposed when the shingle is finally laid, must, of course, be kept intact, and with the present invention that area is protected from adhesion with the superimposed shingle in 75 the bundle by the waxy coating 2, above referred to.

It is conceivable, of course, that the coating might be coextensive of the under face of the shingle, but inasmuch as slight adhesion of that portion of the under face which is adjacent to the tip is not detrimental to the underlying shingle it is found expedient and economical not to coat the entire under face with the waxy substance but to apply 85 such waxy coating transversely of the shingle a distance from the butt equal to or slightly exceeding the area of the part of the underlying shingle of the bundle which is exposed when the same is laid. Another 90 advantage which arises from the treatment as above set forth is that the presence of the waxy material renders the under face of the shingle more nearly waterproof than does the mere presence of the asphaltum or sim- 95 ilar coating. Inasmuch as the water tends to creep upwardly between the overlapping portions of the shingles when laid, the presence of this additional waterproofing material is found of material benefit in tending 100 to prolong the life of the roof.

What is claimed is,—

1. As a new article of manufacture a paper shingle impregnated with asphaltum and having a coating of non-sticky waxy 105 material extending from the butt toward the upper edge of the shingle upon its under face.

2. As a new article of manufacture, a paper shingle impregnated with asphaltum 110 and having its under face coated from the butt toward the upper edge in part at least

with a non-sticky waxy material, the opposite face of the shingle having a finished surface of comminuted stone.

3. As a new article of manufacture, a paper shingle having its under face treated with asphaltum and a coating of Montan wax imposed upon the asphaltum, said coating extending from the butt of the shingle toward the upper edge thereof but stopping 10 short of the upper edge.

4. As a new article of manufacture, a paper shingle having its under face treated with a coating of asphaltum and a layer of non-sticky waterproofing material imposed upon such asphaltum coating from the butt 15 toward the upper edge of the shingle.

In testimony whereof I have signed my name to this specification.

CHARLES S. BIRD.